

## UNITED STATES PATENT OFFICE

2,417,088

## LUBRICATING COMPOSITION

Carl F. Prutton, Cleveland Heights, Ohio, assignor, by mesne assignments, to The Lubri-Zol Development Corporation, Cleveland, Ohio, a corporation of Delaware

No Drawing. Application February 17, 1942,  
Serial No. 431,259

8 Claims. (Cl. 252—48.6)

1

This invention relates, as indicated, to lubricants and more particularly to lubricating compositions and methods of lubricating having certain advantages over such compositions and methods now familiar to those skilled in the art.

This application is a continuation-in-part of my copending application Serial No. 247,000, filed December 21, 1938, which has now issued into Patent No. 2,276,341, which in turn is a continuation-in-part of copending application Serial No. 737,070, filed July 26, 1934, and copending application Serial No. 755,987, filed December 4, 1934.

At the present time there is an increasing demand for lubricating compositions capable of resisting the effects of extreme pressures and temperatures under conditions of use and it is an object of the present invention to provide such a composition.

By "extreme pressures," as referred to above, is meant pressures of or in excess of 10,000 pounds per square inch, such pressures being now commonly encountered in hypoid gears, bearings, contact surfaces of cylinders and piston rings in internal combustion engines, and many other points. Such pressures tend to cause the rupture of the continuous "thick film" of lubricant which separates bearing surfaces under more moderate conditions. A region of "thin film" lubrication results which is also sometimes described as "boundary" lubrication.

A particular object of my invention is, therefore, to provide a lubricant and method of lubricating which will function to advantage under conditions of extreme pressure and effectively prevent seizure and scoring of the relatively moving metallic surfaces being lubricated.

Other objects of this invention will appear as the description proceeds.

To the accomplishment of the foregoing and related ends, this invention, then, comprises the means hereinafter fully described and particularly pointed out in the claims. The following description sets forth in detail certain approved combinations of ingredients embodying my invention, such disclosed means constituting, however, but certain of the various forms in which the principle of the invention may be employed.

Broadly stated, this invention contemplates the use in lubricating compositions of esters of naphthenic acids used either alone or preferably in combination with a separate halogenated organic compound.

When compositions are desired suitable for use in the lubrication of internal combustion engines, it is obvious that only relatively small proportions of these esters should be added to the hydrocarbon base oil. Since, however, it has been found that the presence of even small amounts of these esters will considerably enhance the

10 lubricating properties of mineral lubricating oils especially when employed in combination with separate halogen compounds, liquid compositions are satisfactory for many purposes and may contain as little as 0.1% of the ester although from about 1% to about 5% by weight, based on the amount of oil, is generally more desirable. Amounts up to 20% may be used for certain purposes. Concentrates which may be further blended with base stocks may contain up to as high as 60% of these esters of naphthenic acids.

The base oil employed in the composition of this invention is generally mineral oil but it is to be understood that any other suitable hydrocarbon lubricating oil, whether naturally occurring or synthetic, may be employed as the oil base.

The oil base of the preferred composition of this invention is a highly refined mineral lubricating oil having a viscosity and other characteristics such as to make the same suitable for use as the crankcase lubricant for internal combustion engines. The highly refined mineral lubricating oils suitable for use as the base in 25 the improved compositions of my invention may be conveniently classified in accordance with their viscosity index, three such classes being oils having a V. I. up to 30; oils having a V. I. from 30 to about 70; and oils having a V. I. of above 30 70. Obviously the oil base selected may contain appropriate constituents in addition to plain mineral oil such as pour point depressors and the like, since these conventionally employed materials have been found entirely compatible with the addition agents which characterize the final blends comprising my invention.

It is also within the contemplation of this invention to provide the addition agents in the form of a concentrate in a suitable oil, said oil containing rather high percentages of the addition agents. Such concentrates may be employed for future blending with a lubricating oil in the proportions desired for the particular conditions of use.

The following list of esters suitable for use in accordance with the invention is intended to be illustrative only and it is to be understood that various other compounds coming within the 50 group of esters of naphthenic acids broadly are included within the scope of the invention:

Esters of naphthenic acids:

(1) Aliphatic esters, e. g.,

55 Propyl diiso-propyl naphthenates  
Methyl naphthenate  
Ethyl naphthenate  
Butyl naphthenates (n-, iso-, and sec-)  
Amyl naphthenates  
Lauryl naphthenate  
Cetyl naphthenate

- (2) Aromatic esters, e. g.,  
 Phenyl naphthenate  
 t-Amyl-phenyl naphthenate  
 Benzyl naphthenate  
 Cresyl naphthenate  
 Xenyl naphthenate  
 (3) Cyclo-aliphatic esters, e. g.,  
 Cyclopentyl naphthenate  
 Cyclohexyl naphthenate  
 Methyl-cyclohexyl naphthenates  
 Di-methyl-cyclohexyl naphthenates  
 Tri-methyl-cyclohexyl naphthenates  
 Propyl-cyclohexyl naphthenates  
 Amyl-cyclohexyl naphthenates  
 Lauryl-cyclohexyl naphthenates  
 Cetyl-cyclohexyl naphthenates  
 Cyclohexyl-carbinol naphthenates  
 Cyclohexyl-cyclohexyl naphthenates

Any esters may be used which are derived from naphthenic acids by substituting an organic radicle, R, for the replaceable hydrogen of the acid. Examples of R are the following:

## I. Hydrocarbon radicles:

- (A) Alkyl radicles  
 Amyl (n, iso, sec. and tertiary)  
 Lauryl  
 Cetyl  
 Carnaubyl  
 Ceryl  
 Montanyl  
 M-silsyl  
 Myricyl  
 Lacceryl  
 Psyllcyl

## (B) Aryl radicles

- Phenyl  
 Xenyl  
 Nannthryl (alpha- and beta-)  
 Anthracyl  
 Phenanthryl

## (C) Cyclo-alkyl radicles

- Cycloentyl  
 Cyclohexyl  
 Cycloheptyl  
 Cyclohexyl-cyclohexyl

## (D) Alkylated aryl radicles

- Radicles formed by the alkylation of aryl radicles, such as those listed above (B), with any of the alkyl radicles, e. g., those listed above (A), or with any of the following:  
 Methyl  
 Ethyl  
 Propyl (n-, and iso-)  
 Butyl (n-, iso- and sec.)

Specific examples of alkylated aryl radicles are as follows: 45

- Cresyl  
 Xyl  
 Trimethyl-phenyl  
 Ethyl-phenyl  
 Tetra-ethyl-phenyl  
 t-Amyl phenyl  
 Lauryl-phenyl  
 Cetyl-phenyl  
 Methyl-naphthyl  
 Iso-propyl-naphthyl  
 t-Amyl-naphthyl  
 Lauryl-naphthyl  
 Cetyl-naphthyl  
 Iso-propyl-xenyl  
 t-Amyl-xenyl  
 Lauryl-xenyl

## (E) Alkylated cyclo-alkyl radicles

- Radicles formed by the alkylation of cyclo-alkyl radicles, such as those listed above (C), with any of the alkyl radicles, such as those listed above. Specific examples are:

- Methyl-cyclohexyl  
 Dimethyl cyclohexyl  
 t-Amyl cyclohexyl  
 Lauryl cyclohexyl  
 Cetyl cyclohexyl

## (F) Cyclo-alkylated aryl radicles, e. g.

- Cyclohexyl-phenyl  
 Cyclohexyl-xenyl  
 Cyclohexyl-naphthyl

## (G) Arylated-alkyl radicles, e. g.

- Benzyl  
 Phenyl-ethyl  
 Phenyl-amyyl  
 Phenyl-lauryl  
 Phenyl-cetyl  
 Xenyl-methyl  
 Xenyl-ethyl  
 Naphthyl-methyl  
 Naphthyl-ethyl  
 Naphthyl-cetyl

## (H) Cyclo-alkylated alkyl radicles, e. g.

- Naphthyl  
 Hexahydrobenzyl  
 Cyclohexyl-ethyl  
 Cyclohexyl-amyyl

- I. Hydrocarbon radicles—Continued:  
 (I) Arylated cyclo-alkyl radicles, e. g.  
 Phenyl-cyclohexyl  
 Xenyl-cyclohexyl  
 Naphthyl-cyclohexyl

- 5 (J) Mixed radicles, e. g.  
 Methylcyclohexyl-phenyl  
 Amylcyclohexyl-phenyl  
 Cyclohexyl-cresyl  
 Cyclohexyl-xyl  
 Cyclohexyl-amyyl-phenyl  
 Cyclohexyl-benzyl  
 Xyl-cyclohexyl  
 Lauryl-phenyl cyclohexyl  
 Cetyl-phenyl cyclohexyl  
 Phenyl-methylcyclohexyl  
 Phenyl-amylcyclohexyl  
 Xyl-methylcyclohexyl  
 Benzyl-cyclohexyl  
 Benzyl-methylcyclohexyl  
 Methylcyclohexyl-amyyl  
 Methylcyclohexyl-lauryl

## II. Oxygen-containing organic radicles

- (A) Of the ether type, e. g.  
 Methoxy-phenyl  
 Ethoxy-phenyl  
 Lauroxy-phenyl  
 Cyclohexoxy-phenyl  
 Phenoxy-phenyl  
 Phenoxyl-naphthyl  
 Phenoxy-cyclohexyl  
 Phenoxy-ethyl  
 Phenoxyl-lauryl  
 Phenoxy-cetyl  
 Amyl-phenoxy-ethyl  
 Phenyl-ethoxy-ethyl  
 $-C_2H_5-O-C_2H_5$ —(derived from di-ethylene glycol)

## (B) Of the ketone type, e. g.

- Acetyl-phenyl  
 Acetyl-xenyl  
 Acetyl-naphthyl  
 Acetyl-lauryl  
 Acetyl-cetyl  
 Acetyl-cyclohexyl  
 Acetyl-naphtheneyl  
 Lauroyl-phenyl  
 Benzoyl-phenyl  
 Benzoyl-naphthyl  
 Benzoyl-cyclohexyl  
 Benzoyl-naphtheneyl  
 Benzoyl-lauryl  
 Benzoyl-cetyl  
 Stearoyl-phenyl  
 Stearoyl-xenyl  
 Stearoyl-naphthyl  
 Stearoyl-amyyl  
 Stearoyl-lauryl  
 Stearoyl-cetyl  
 Stearoyl-phenoxyphenyl  
 Stearoyl-cyclohexyl  
 Stearoyl-naphtheneyl  
 Naphthenoxy-phenyl  
 Naphthenoxy-xenyl  
 Naphthenoxy-naphthyl  
 Naphthenoxy-amyyl  
 Naphthenoxy-lauryl  
 Naphthenoxy-cetyl  
 Naphthenoxy-phenoxyl-phenyl  
 Naphthenoxy-cyclohexyl  
 Phenoxybenzoyl-phenyl

## (C) Of the ester type, i. e.

Derived from hydroxy-esters by the removal of the hydroxyl group, as for example, by the removal of the hydroxyl group from the following esters:

- (1) Esters of hydroxy acids, e. g., esters formed by substitution of any of the "R" groups listed above for one or more of the acid hydrogen atoms of the following acids:

- Lactic acid  
 Hydroacrylic acid  
 Citric acid  
 Tartaric acid  
 Ricinoleic acid  
 Hydroxy-stearic acid  
 Hydroxy-chlorstearic acid  
 Cyclohexanol carboxylic acids  
 Hydroxybenzene acids  
 Salicylic acid  
 Hydroxy-phthalic acids  
 Hydroxy-phenyl-benzoic acids  
 Naphthol carboxylic acids

- (2) Esters of polyhydroxy alcohols and phenols in which at least one hydroxyl group remains unsubstituted, for example—esters formed by esterifying the following so that at least one hydroxyl group remains in the resulting ester:

- Ethylene glycol  
 Diethylene glycol  
 Propylene glycols  
 Butylene glycols  
 Poly-hydroxy benzenes  
 Dihydroxy-benzenes  
 Resorcinol  
 Catechol  
 Hydroquinone  
 Tri-hydroxybenzenes  
 Pyrogallol

III. Sulphur-containing radicles, e. g. any of the examples of oxygen-containing radicles in which at least one oxygen atom has been replaced with sulphur. Specific examples of sulphur-containing radicles are:

(A) Of the thio-ether type

Thio-phenoxy-phenyl ( $C_6H_5-S-C_6H_5-$ )  
Thio-phenoxy-ethyl ( $C_6H_5-S-C_2H_5-$ )  
Thio-lauroyl-phenyl ( $C_{11}H_{23}-S-C_6H_5-$ )  
Thio-t-amyl-phenoxy-phenyl  
( $C_3H_11-C_6H_5-S-C_6H_5-$ )  
Thio-t-amyl-phenoxy t-amyl-phenyl



(B) Of the thio-ketone type

Thio-acetyl-phenyl  
Thio-benzoyl-phenyl  
Thio-stearyl-phenyl  
Thio-naphthenoyl-phenyl  
Thio-stearyl-cyclohexyl

(C) Of the thio-ester type, e. g., derived from hydroxy-esters of thio-carboxylic acids. Examples of such radicles are:



Where R is methyl, ethyl, butyl, amyl, lauryl, stearyl, naphthyl, etc.

(D) Radicles derived from hydroxy-organic polysulphides by removal of the hydroxy group, e. g.



where R is hydrogen or an alkyl or cyclo-alkyl group

R-Sn-R'

where R is an alkyl or cyclo-alkyl group and R' is an alkylene group.

As previously indicated, this invention comprises the use in lubricating compositions of esters of naphthenic acid. These esters, when used alone, that is, without any other addition agent effective to cooperate therewith, are admirably suited to impart to the lubricant to which they are added, properties such as oiliness, reduction in rate of wear which enables such lubricant to be used under conditions where the plain refined mineral lubricating oil base would be unsatisfactory for use alone.

These esters of naphthenic acid, which may be used alone, may be either the straight esters or such esters halogenated, and accordingly this invention comprises the use in lubricating compositions of both the halogenated and unhalo-

genated esters of naphthenic acids. The specific examples previously given are the unhalogenated esters which may be thus used. Each of the esters thus identified, either generically, sub-generically or specifically, may be modified by halogenation, and the halogenated ester thus derived used as the addition agent.

It is believed unnecessary to repeat the foregoing list in the more specific identification of the 10 halogen-bearing esters, since it will be obvious to those skilled in the art what the halogen counterparts of these esters would be. The usual halogenation process, well-known to those familiar with the art, may be employed in the preparation of the halogenated esters. The usual halogenation step may be followed by subsequent stabilization treatments, such as air blowing, alkali washing, or the like, in order that the halogen retained in the ester will be sufficiently stable, and not 15 too readily liberated during storage and use.

The following, however, is a list of specific examples of halogen-bearing esters of naphthenic acids which will be found particularly suitable and this, therefore, constitutes a preferred group 20 of compounds for use in the lubricating compositions of my invention.

Chlorinated methyl naphthenate containing about 20% chlorine

30 Chlorinated butyl naphthenate containing about 10% chlorine

Chlorinated methyl-cyclohexyl naphthenate containing about 10% chlorine

Chlorinated methyl-cyclohexyl naphthenate containing about 40% chlorine

35 Chlorphenyl naphthenates

Chlorbenzyl naphthenates

Dichlorbenzyl naphthenates

Dichlor-xenyl naphthenates

Tetra-chlor-xenyl naphthenates

40 Tetra-chlor-phenoxy-phenyl naphthenates

Hexachlor-phenoxy-phenyl naphthenates

This invention thus contemplates the utilization of halogen in combination with the esters 45 of naphthenic acid. The halogen may be, as indicated above, included in the same molecule as by halogenation of the ester, itself, or the halogen may be present in a separate molecule, i. e. a separate halogen-bearing organic compound. It

50 has been found that the esters of naphthenic acid have a cooperative effect when employed in conjunction with a separate halogenated organic compound. This is true whether the naphthenic acid ester be halogenated or unhalogenated. This cooperation between the naphthenic acid esters and the separate organic halogen compound is manifested by the ester cooperating with the separate halogen compound in activating the latter, so that a higher film strength may be attained from the use of a given amount of halogen in the form of the separate organic halogen compound, and moreover, extremely stable halogenated organic compounds, which would have a low degree of activity, may be rendered especially active by the incorporation therewith of an ester of naphthenic acid, whether the latter be halogenated or unhalogenated.

This invention, therefore, includes the combined use of the esters of naphthenic acids, either 60 halogenated or unhalogenated, with a separate organic halogen compound, and this combination, for the reasons above given, is the preferred embodiment of my invention, since in such combination, the greatest utility of the esters of naphthenic acids may be realized.

For purposes of classification, the halogenated organic compounds, which thus comprise one component of the preferred embodiment of my invention, may be conveniently grouped as "oxygen-free" and "oxygen-bearing."

In the case of the halogenated aromatic oxygen-free compounds, it is preferable for certain uses that the halogen be attached to a carbon atom of the benzenoid ring. These latter compounds are sometimes more desirable because of their non-corrosive character and general stability.

The halogenated oxygen-free organic compounds as noted may be either:

- A. Aliphatic, such as halogenated:
  - I. Hydrocarbons, notably, those containing from four to ten carbon atoms, e. g.,
    - Chlorinated or fluorinated hexane
    - Chlorinated or fluorinated octane
    - Chlorinated or fluorinated decane
  - II. Amines, primary, secondary and tertiary, e. g., hexylamines, di-aminamines, tri-aminamines such as:
    - Chlorinated or fluorinated tri-ethyl amine
    - Chlorinated or fluorinated hexyl amines
  - Also:
    - Chlorinated or fluorinated tributyl amine
  - III. Nitriles
    - Halogenated ethyl nitrile
    - Halogenated butyl nitrile

or (preferable for certain types of uses as noted above):

- B. Cyclic compounds, such as halogenated:
  - I. Benzene and related compounds such as:
    - (1) Halogenated benzene, e. g.,
      - The dichlorbenzenes, notably the ortho compound
      - Ortho-dibrom benzene
      - The fluorinated benzenes
    - (2) Halogenated derivatives of benzene such as:
      - (a) Halogenated homologs of benzene, e. g.,
        - Mono-chlor toluene
        - Mono-chlor xylene
        - Mono-chlor cymene
        - Ethyl mono-chlor benzenes
        - Propyl mono-chlor benzenes
        - Di-ethyl mono-chlor benzenes
        - Ethyl dichlor benzenes
        - Propyl dichlor benzenes
        - Di-ethyl dichlor benzenes
        - Di-ethyl tetrachlor benzenes
      - (b) Halogenated amino derivatives of benzene, e. g.,
        - Chlorinated aniline
        - Mono-chlor aniline (preferably the ortho compound)
        - Mono-chlor di-methyl aniline
        - Chlorinated toluidines
        - Chlorinated xylylides
        - Chlorinated diphenylamine
      - (c) Halogenated hydrobenzenes, e. g.,
        - Di-chlor hydrogenated-benzenes such as
        - Dichlorhexahydrobenzene
        - (dichlor cyclohexane)
      - (3) Halogenated aromatic nitriles, e. g.,
        - Chlorinated phenyl nitrile
    - II. Polyphenyls, and related compounds, including diphenyl, diphenyl benzenes, etc., such as,
      - (1) Chlorinated diphenyl, e. g.,
        - Mono-chlor diphenyls
        - Di-chlor diphenyls
        - Tri-chlor diphenyls
      - (2) Brominated diphenyl, e. g.,
        - The mono-brom diphenyls
      - (3) Fluorinated diphenyl
      - (4) Halogenated derivatives of diphenyl, such as,
        - (a) Halogenated homologs of diphenyl, e. g.,
          - Chlorinated methyl diphenyls
          - Chlorinated ethyl diphenyls
        - (b) Halogenated amino derivatives of diphenyl, e. g.,
          - Chlorinated amino-diphenyls
          - Chlorinated amino methyl diphenyls
        - (c) Halogenated hydrodiphenyls, e. g.,
          - Chlorinated phenyl hexahydrobenzene
          - Chlorinated dodecahydronaphthalene
    - III. Naphthalene, such as
      - (1) Chlorinated naphthalene, e. g.,
        - $\alpha$ -Mono-chlor naphthalene
      - (2) Brominated naphthalenes, e. g.,
        - $\alpha$ -Monobrom naphthalene
      - (3) Fluorinated naphthalene
      - (4) Halogenated derivatives of naphthalene such as:
        - (a) Halogenated homologs of naphthalenes, e. g.,
          - Chlorinated methyl naphthalene notably the alpha compound, chlorinated propyl, and isopropyl substitution products of naphthalene
        - (b) Halogenated amino derivatives of naphthalene, e. g.,
          - Chlorinated naphthylamines
          - Mono-chlor  $\alpha$ -naphthyl amine
        - (c) Halogenated hydronaphthalenes, e. g.,
          - Chlorinated decahydronaphthalene

Cyclic compounds, such as halogenated—Continued:  
IV. Phenanthrene and anthracene and related compounds, such as:

- (1) Chlorinated phenanthrene, chlorinated anthracene
- (2) Halogenated derivatives of phenanthrene and anthracene, such as:

- (a) Halogenated homologs
  - Chlorinated 1-methyl phenanthrene
  - Chlorinated 3-methyl phenanthrene
  - Chlorinated 9,10 dimethyl phenanthrene
  - Chlorinated propyl and isopropyl derivatives of phenanthrene
  - Chlorinated dimethyl anthracenes
  - Chlorinated  $\alpha$ -methyl anthracene
  - Chlorinated  $\beta$ -methyl anthracene
  - Chlorinated propyl and isopropyl derivatives of anthracene

- (b) Halogenated amino derivatives, e. g.,
  - Chlorinated phenanthryl amines
  - Chlorinated anthramines

- (c) Halogenated hydrophenanthrenes and halogenated hydroanthracenes, e. g.,
  - Chlorinated retene oil (contains hydro retene)

V. Chrysene, picene, and related compounds, including their derivatives, such as homologs, amino derivatives and other substitution products.

VI. Bridged ring compounds, such as the terpenes and related compounds, and their derivatives, e. g., chlorinated pinene.

VII. Heterocyclic compounds, such as pyridine, quinoline pyrrole, thiophene, and derivatives of them, e. g., monochlor pyridine.

Very satisfactory results may be obtained when two or more different halogens are present in the same molecule, orthobrom-chlor benzene, ethyl-bromochlor benzenes, and the fluorinated chlorine compounds being good examples of such compounds. If the aromatic compounds have been alkylated they are often especially effective.

As a matter of convenience, the halogenated di-phenyls and substituted diphenyls, as well as halogenated substituted benzenes where two or 35 more phenyl groups are directly linked, may be inclusively referred to as halogenated poly-phenyls.

Some of the best examples of the aromatic compounds are:

- Chlorinated benzene, B—I. (1) e. g.,
  - Di-chlor benzene (notably the ortho compound)
- Mono-chlor toluene, B—I. (2) (a)
- Oi-ethyl tetrachlor benzene
- Chlorinated diphenyl B—II (1)
- Chlorinated aniline B—I (2) (b)
- Chlorinated pyridine B—VIII.
- Chlorinated quinoline B—VII.

Good examples of halogenated aliphatic hydrocarbons are:

- Fluorinated pentane
- Fluorinated hexane
- Fluorinated octane
- Fluorinated di-iso-butene
- Halogenated petroleum derivatives, particularly halogenated petroleum oils and waxes.

#### 60 Halogenated oxygen bearing organic compounds

Here, as above, compounds of the aromatic series with the halogen attached to the ring are favored for purposes in which it is desirable to have the halogen present in its most stable combined form. However, for certain uses the halogenated oxygen-bearing aliphatic compounds have been found to be more effective and satisfactory.

70 The oxygen-bearing compounds may, for convenience, be classified as follows:

- I. Aliphatic, or carbon chain type.—Oxygen-bearing derivatives of:
  - A. Hydrocarbons of the paraffin series,
  - B. Hydrocarbons of the olefinic series and
  - C. Hydrocarbons of the acetylene series.

## II. Organic ring type.—Oxygen-bearing derivatives of:

## A. "Carbon ring" type compounds

- (a) Of the aromatic, or allied type, including oxygen-bearing derivatives of benzene, naphthalene, anthracene, etc., also compounds of the bridged ring type, such as the terpenes, and related compounds.
- (b) Of the class including the cycloparaffins, cycloolefines, etc. Examples of this class are oxygen-bearing derivatives of the following:
- (1) Hydrogenation products of benzene (e. g., cyclohexane, cyclohexene, cyclohexadiene); such as hydrogenated phenol, notably: cyclohexanol, di-hydro-phenol, tetra-hydro-phenol.
  - (2) Hydrogenation products of naphthalene (e. g., decahydronaphthalene, tetrahydronaphthalene, etc.); such as the hydrogenated naphthols.
  - (3) Naphthalenes, such as naphthenic acid, etc.

- (c) Of mixed type such as derivatives of indene, 15 hydrindene, hydranthracene, etc.

## B. "Heterocyclic" type compounds

- (a) Of the aromatic or allied type including derivatives of pyridine, quinoline, etc.
- (b) Other types such as furfural, furan and its derivatives and derivatives of thiophene, pyrrole, etc.

The oxygen-bearing derivatives of the foregoing compounds may also be classified according to the nature of the attachment of the oxygen to the molecule, viz.:

## I'. Directly attached to one or more carbon atoms, as in the case of:

- (1') Ethers and analogous compounds
- (2') Compounds containing the



radicle, such as alcohols and other derivatives of carbinol (including phenols, cresols, naphthols, etc.)

- (3') Compounds containing the carbonyl



radicle, such as amides, aldehydes, ketones, organic acids, esters and salts of organic acids, thio-acids and esters of thio-acids

- (4') Compounds in which oxygen forms a part of the ring structure, e. g., furan and its derivatives, etc.
- (5') Compounds with inorganic radicle where the oxygen is directly attached to carbon atom

Ar-sulfite  
Hypochlorite  
Phosphite  
Thiophosphate  
Thiophosphite  
 $\beta$ -hydroxyamines

## II'. Indirectly attached through the means of some other atom, i. e., in the form of an inorganic radicle, e. g.:

- Ar-sulfate  
Chlorate  
Chlorite  
Chlorite  
Cyanate  
 $\alpha$ -hydroxylamine  
Nitrate  
Nitrite  
Nitro  
Nitroso  
Oxime  
Perchlorate  
Phosphate  
Sulphate  
Sulphite  
Sulphite  
Sulphonic acid  
Sulphone  
Sulphonic acid  
Sulphoxide  
Thio-sulphate

The following table indicates some of the compounds which are particularly suitable for use in accordance with the present invention:

## A. Aromatic

- (1) Phenols, e. g.,  
o-Chlor phenol  
Monochlor  $\alpha$ -naphthols
- (2) Alcohols, e. g.,  
The chlor-benzyl alcohols
- (3) Ketones, e. g.,  
Mono chlor benzophenones  
Chlor naphthyl ketones  
Chlor-methyl-benzophenones
- (4) Acids, e. g.,  
Chlorophenyl acetic acids  
Chlor salicylic acids  
Chlor phenyl stearic acids
- (5) Esters, e. g.,  
Methyl chlorbenzoates  
Ethyl chlorbenzoates  
Butyl chlorbenzoates  
Dimethyl chlorphthalates  
Di-ethyl chlorphthalates  
Dibutyl chlorphthalates  
Methyl chlor salicylates  
Methyl chlor-phenyl-stearates

## A. Aromatic—Continued:

- (6) Ethers, e. g.,  
Chlorinated diphenyl ether  
Chlorophenyl ethyl ethers  
Chlorinated dixenyl ether  
Chlorinated dinaphthyl ether  
Alkylated chlor-diphenyl ethers
- (7) Non-aromatic oxygen-bearing organic ring compounds:  
Halogenated cyclohexanol  
Halogenated esters of naphthenic acids
- (8) Oxygen-bearing heterocyclic compounds:  
(a) Halogenated furane and derivatives of furane, e. g.,  
Halogenated esters of pyrrolinic acid (furoates)  
Halogenated furfuryl alcohol and esters of it, e. g.,  
Chlorinated furfuryl acetate
- (b) Halogenated oxygen-bearing derivatives of thiophene and pyrrole, e. g.,  
Chlorinated esters of thiophene  
Carboxylic acids and chlorinated  
Esters of pyrrole carboxylic acids

## B. Chain compounds

- (1) Alcohols  
Fluorinated octyl alcohol  
Fluorinated decyl alcohol  
Fluorinated lauryl alcohol  
Fluorinated cetyl alcohol
- (2) Esters  
Methyl dichlorstearate  
Chlorinated tri-lauryl phosphate  
Chlorinated tri-ethyl phosphate
- (3) Ketones  
Chlorinated dibutyl ketone  
Chlorinated di-amyl ketone

It is, of course, to be understood that the above lists of compounds are intended merely to illustrate the type of compound suitable as one component of the addition agent of this invention and are not to be construed as limiting said component to the particular groups or examples there disclosed.

It is believed that under conditions of extreme pressure the halogenated addition agents of this invention react chemically or physico-chemically with the metallic surfaces to form a non-fluxing surface which will not seize or score. This invention is not intended to be limited, however, by any particular theory or explanation of the action upon the metallic surfaces.

All of the various halogens are effective when employed in accordance with the present invention but chlorine is generally preferred inasmuch as it is the least expensive and one of the most effective of the halogens. Bromine and fluorine are more expensive and the latter is relatively difficult to handle but they are each usable in accordance with this invention. Iodine is not so readily obtainable as the other halogens and is quite expensive but it also is satisfactory in providing effective addition agents. It should also be noted that two or more different halogens may be present in the same molecule. The brom-chlor and fluorinated chlorine or bromine compounds give especially satisfactory results. When used in conjunction with a naphthenate, an amount of from about 0.1% to about 20% by weight, based on the amount of oil, of the separate halogen compound is all that is required to render the finished lubricant efficient under conditions of extreme pressure. Seldom is there any need to employ more than 10% and usually about 3% of the halogenated addition agent will be found to be ample for most purposes.

Since, in general, the loss of the addition agent by volatilization will be less for compounds having a low volatility, the vapor pressure of the compounds should, for most purposes, be less than atmospheric pressure at temperatures up to 140° C. It is usually desirable, especially for use in internal combustion engines, that the vapor pressure be less than atmospheric at temperatures up to 170° C. In the case of compounds which are stable at temperatures up to their boiling points, this condition may be expressed by stating that the boiling point of the compound should, in general, be higher than 140° C., and for certain uses,

such as in internal combustion engines, higher than 170° C.

While mineral oil generally is the principal ingredient of the lubricant, it is not essential that it be the only ingredient other than the addition agent, provided that there be no additional ingredient which is incompatible with such addition agent. It is within the contemplation of this invention to include, if necessary or desirable, such other addition agents as are commonly added to improve the viscosity index or cold test of the lubricant and a lubricating composition according to this invention which also has a separate oiliness increasing agent has been found to be especially effective.

As illustrative of specific embodiments of my invention I will list below a number of specific examples of final blends which, it will be noted, are divided into two groups, the first group being motor oils adapted for use in the crankcases of internal combustion engines, and the second group being gear oils useful, for example, in the gearcases of automobiles and the like.

#### I. Motor oils

|                                                                         | Per cent |
|-------------------------------------------------------------------------|----------|
| 1. Mineral oil                                                          | 99.5     |
| Chlorinated methyl naphthenate containing about 20% chlorine            | .5       |
| 2. Mineral oil                                                          | 99.5     |
| Chlorinated methyl cyclohexyl naphthenate containing about 10% chlorine | .5       |
| 3. Mineral oil                                                          | 99       |
| Dichlorobenzyl naphthenate                                              | 1        |
| 4. Mineral oil                                                          | 98.5     |
| Ortho dichlorbenzene                                                    | 1.0      |
| Methyl naphthenate                                                      | .5       |
| 5. Mineral oil                                                          | 98.5     |
| Chlorinated diphenyl containing about 50% chlorine                      | 1.0      |
| Butyl naphthenate                                                       | .5       |
| 6. Mineral oil                                                          | 98.5     |
| Ortho dichlorbenzene                                                    | .5       |
| Hexadichloridiphenyl ether                                              | .5       |
| Methyl naphthenate                                                      | .5       |
| 7. Mineral oil                                                          | 98.75    |
| Ortho dichlorbenzene                                                    | .5       |
| Hexachlor diphenyl ether                                                | .5       |
| Chlorinated methyl naphthenate containing about 20% chlorine            | .25      |

The "mineral oil" given in the foregoing list of compositions Nos. 1 to 7 inclusive, may be any suitable highly refined mineral lubricating oil having characteristics suiting the same for use as a crankcase lubricant. For example, the "mineral oil" used in each of Examples 1 to 7 may be an S. A. E. 20 Pennsylvania motor oil having a viscosity index of about 100. As previously indicated, this "mineral oil" may include, in addition to highly refined mineral lubricating oil, other constituents such as pour point depressors and the like. The S. A. E. number may, of course, vary in accordance with the usual standards which are observed in fitting an oil base to a particular use or condition of use.

#### II. Gear oils

|                                                                         | Per cent |
|-------------------------------------------------------------------------|----------|
| 8. Mineral oil                                                          | 93       |
| Chlorinated methyl cyclohexyl naphthenate containing about 40% chlorine | 7        |

|                                                                                                                                                         | Per cent |
|---------------------------------------------------------------------------------------------------------------------------------------------------------|----------|
| 9. Mineral oil                                                                                                                                          | 92.5     |
| Chlorinated paraffin wax containing about 40% chlorine                                                                                                  | 7.0      |
| Methyl naphthenate                                                                                                                                      | .5       |
| 10. Mineral oil                                                                                                                                         | 91       |
| Chlorinated paraffin wax containing about 40% chlorine                                                                                                  | 8        |
| Methyl naphthenate                                                                                                                                      | 1        |
| 11. Mineral oil                                                                                                                                         | 91.75    |
| Chlorinated paraffin wax containing about 40% chlorine                                                                                                  | 8.00     |
| Chlorinated methyl naphthenate containing about 20% chlorine                                                                                            | .25      |
| 12. Mineral oil                                                                                                                                         | 89.8     |
| Chlorinated paraffin wax containing about 40% chlorine                                                                                                  | 7.0      |
| Chlorbenzyl disulphide                                                                                                                                  | 3.0      |
| Methyl cyclohexyl naphthenate                                                                                                                           | .2       |
| 13. Mineral oil                                                                                                                                         | 89.9     |
| Chlorinated paraffin wax containing about 40% chlorine                                                                                                  | 8.0      |
| Benzyl disulphide                                                                                                                                       | 2.0      |
| Chlorinated methyl naphthenate containing about 20% chlorine                                                                                            | .1       |
| 14. Mineral oil                                                                                                                                         | 89       |
| Reaction product of chlorinated paraffin wax, containing about 35% chlorine, with sodium disulphide, such reaction product containing about 20% sulphur | 10       |
| Methyl naphthenate                                                                                                                                      | 1        |
| 15. Mineral oil                                                                                                                                         | 89.5     |
| Reaction product of chlorinated paraffin wax, containing about 35% chlorine, with sodium disulphide, such reaction product containing about 20% sulphur | 10.0     |
| Chlorinated methyl cyclohexyl naphthenate containing about 10% chlorine                                                                                 | .5       |

The "mineral oil" identified a component in each of compositions 8 to 15 inclusive is preferably a gear oil suitable for use as the base in lubricants designed for use in gearcases. For example, an entirely satisfactory composition may be produced by utilizing as the "mineral oil" component in each of compositions 8 to 15 inclusive an S. A. E. 90 gear oil having a viscosity index of about 70. Here again, the "mineral oil" component may include not only a refined mineral lubricating oil of properties such as those given above, but may also include other components such as thickening agents and the like.

Attention is directed particularly to Examples 12 to 15 above which are additionally characterized by the presence therein of an organic sulphur compound which, in certain instances, such as for example composition No. 12, may contain chlorine in the same molecule with the sulphur. This combination, i. e., the combination of an ester of a naphthenic acid with an organic sulphur compound, and with or without a separate organic halogen compound, has been found to be of particular utility. The organic sulphur compound and the esters of naphthenic acid, whether halogenated or unhalogenated, cooperate in the production of a final lubricating composition characterized by properties such as oiliness, film strength, and ability to reduce wear, which it is not possible to achieve with the use of either of these components alone, and which is more than

the cumulative effect of such components when used separately.

Other modes of applying the principle of my invention may be employed instead of the one explained, change being made as regards the materials employed, provided the ingredients stated by any of the following claims or the equivalent of such stated ingredients be employed.

I, therefore, particularly point out and distinctly claim as my invention:

1. A lubricating composition comprising the combination of an ester of a naphthenic acid and an organic sulphur compound.

2. A lubricating composition comprising a hydrocarbon oil and minor amounts of both an ester of naphthenic acid and a separate organic compound containing an element of the class consisting of halogen and sulphur.

3. A lubricating composition comprising the combination of an ester of a naphthenic acid and an organic halogen compound having a vapor pressure less than atmospheric at 140° C.

4. A lubricating composition comprising a hydrocarbon oil, a halogenated organic compound, and from about 0.1% to about 5% by weight, based on the amount of oil, of an ester of a naphthenic acid.

5. A lubricating composition comprising a hydrocarbon oil, a halogenated organic ring compound, and from about 0.1% to about 5% by weight, based on the amount of oil, of an ester of a naphthenic acid.

6. A lubricating composition comprising a hydrocarbon oil, from about 0.1% to about 5% of an oil-soluble ester of a naphthenic acid, and a stable oil-soluble halogenated organic compound, said compound having a vapor pressure less than

atmospheric at 140° C., and present in an amount less than 10% based on the amount of mineral oil but sufficient to provide a lubricating composition effective to prevent seizure and scoring of relatively moving metallic surfaces under pressure substantially in excess of 10,000 pounds per square inch.

7. A lubricating composition comprising the combination of an ester of a naphthenic acid and a chlor benzyl sulphide.

8. A lubricating composition comprising the combination of methyl naphthenate and a chlor benzyl sulphide.

CARL F. PRUTTON.

15

#### REFERENCES CITED

The following references are of record in the file of this patent:

20

| Number    | Name     | Date          |
|-----------|----------|---------------|
| 2,276,341 | Prutton  | Mar. 17, 1942 |
| 2,224,541 | Frolich  | Dec. 10, 1940 |
| 2,121,976 | Mikeska  | June 28, 1938 |
| 1,882,816 | Hagedorn | Oct. 18, 1932 |
| 2,135,092 | Maverick | Nov. 1, 1938  |

#### UNITED STATES PATENTS

25

| Number  | Country | Date          |
|---------|---------|---------------|
| 402,262 | British | Nov. 30, 1933 |

30

#### FOREIGN PATENTS

35

|                                                                        |
|------------------------------------------------------------------------|
| Industrial and Engineering Chemistry, vol. 28, #10, Oct. 1936.         |
| Article by Lincoln et al., pages 1191-1197. (Copy in Div. 64.) 252-58. |

#### OTHER REFERENCES